

Feb. 9, 1937.

F. L. CHASE

2,070,330

REFRIGERATING APPARATUS

Filed Aug. 31, 1931



Fig. 1



Fig. 3



Fig. 5



Fig. 2



Fig. 4

INVENTOR  
Frederic L. Chase.  
BY  
Spencer, Hardman, and Fahr.  
HIS ATTORNEYS.

## UNITED STATES PATENT OFFICE

2,070,330

## REFRIGERATING APPARATUS

Frederic L. Chase, Dayton, Ohio, assignor, by  
mesne assignments, to General Motors Cor-  
poration, a corporation of Delaware

Application August 31, 1931, Serial No. 560,337

6 Claims. (Cl. 154—28)

This invention relates to refrigerating apparatus and more particularly to a method of manufacturing heat insulated wall structures for use in the manufacture of refrigerating cabinets.

5 One of the most important problems connected with the manufacture of refrigerator cabinets is the provision of means for excluding moisture from accumulating within the confines of the wall structure, for example, within the insulating material itself or on the surface of the cold liner. The tendency for moisture to condense within the wall structure is obviously inherent in all such cabinet constructions for since the interior of the cabinet is maintained at a temperature consider- 10 ably lower than the temperature of the surrounding atmosphere, there is quite a large temperature gradient between the interior and exterior walls of the cabinet. On this gradient and conse- quently within the wall structure there occurs a 15 temperature called the dew point, at which point the moisture in the air tends to condense. Such condensation is detrimental to the long life of the cabinet structure for it not only increases the heat conductivity of the wall but also tends to 20 break down the insulating structure itself.

With these difficulties in mind, it has been the practice heretofore to attempt to waterproof the wall structures to prevent the passage of water vapor from the surrounding atmosphere to the 25 point at which condensation takes place. For this purpose it has been the practice to apply asphaltic material such as a pitch-like bituminous compound known to the trade under various names, one of which is hydrolene, to the walls 30 of the cabinet and insulating material. Hereto- fore, this asphaltic treatment has not been satis- 35 factory and in practically all cases of unsatisfactory results, the trouble has been caused by improper methods of applying the asphaltic 40 material to the insulation.

It is the purpose and object of my present invention to overcome the defects of prior methods of applying asphalt to insulating material by controlling the conditions governing the applica- 45 tion of the asphalt, particularly the tempera- ture at which the asphalt is applied.

In order to more clearly disclose my invention, I have illustrated certain wall structures on the 50 attached drawing.

Further objects and advantages of the present invention will be apparent from the following description, reference being had to the accom- 55 panying drawing, wherein a preferred form of the present invention is clearly shown.

In the drawing:

Fig. 1 is a sectional view of a refrigerator cabinet embodying features of my invention, the section being taken on a line beyond the door opening;

Fig. 2 is a sectional view of a second cabinet showing additional features, the section being likewise taken on a line beyond the door opening;

Fig. 3 is a diagrammatic section of a wall structure showing the results of one manner of applying the asphaltic material;

Fig. 4 is a diagrammatic section of a wall structure showing the results of a second manner of applying the asphaltic material, and

Fig. 5 is a diagrammatic section of the results of a third set of operating conditions.

In order to illustrate my invention and the importance it plays in the manufacture of heat insulated refrigerator cabinets, I have disclosed in Figs. 1 and 2, refrigerator cabinets. These 20 cabinets are shown as having a frame structure composed of wood corner post members 10 and carried by said frame and an inner metal lining 11, and an outer metal covering 12 with a block or slab of corkboard or rock cork 14 therebetween. 25 In such a construction the lining 11 bounding the cold compartment is relatively cold and tends to draw and condense moisture from the warmer outside atmosphere into and within the insulating slab 14. For this reason, the insulating slab 14 30 is sealed against the ingress of moisture from the warmer atmosphere by means of asphaltic material. As shown in Fig. 1, the insulating material may be sealed by a layer of asphaltic material 16 between the lining 11 and the slab 14 and around 35 the outer surfaces of the slab 14, or, as shown in Fig. 2, the asphalt 16' may be only on the external exposed surfaces of the insulating material.

The particular methods by which the cabinets are assembled and the insulation is sealed there- 40 on are not of importance as far as my invention is concerned. For example, the cabinet may be assembled and the insulation sealed by first applying a layer or coating of asphalt to the out- side surface of the inner lining 11, coating one 45 side of the insulating slab and pressing the coated slab against the lining. Asphalt may then be poured onto the outer surface of the insulation to produce the structure disclosed in Fig. 1. Or, if the structure disclosed in Fig. 2 is desired, the 50 slab 14 is placed on the liner 11 and the layer of asphalt sprayed or painted on the outside sur- face thereof. Still another method would be as- sembling the inner and outer walls 11 and 12 55 with the insulation therebetween and subsequently

pouring in the asphalt in a molten condition between the lining 11 and insulation 14 and/or between the outer wall 12 and the insulating slab.

Heretofore, all attempts at sealing the insulating material by means of asphalt have been unsatisfactory for the reason that the conditions governing the application of the asphalt have not been correctly controlled.

I have found that the temperature at which the asphalt is applied is most important. For example, if the temperature at which a specific asphaltic compound is applied is too high, then the degree of penetration of the asphalt into the block of insulating material is too great, thereby 10 improperly sealing the slab against the ingress of moisture and consequently resulting in a poor construction as set forth above.

Such a condition is clearly shown in Fig. 3, wherein it is apparent that the asphalt indicated at 40 has penetrated to great depths in the insulating material 14. Since the insulating properties of asphalt are not as good as those of corkboard, it follows that the insulating effect of the corkboard has been decreased. It is also apparent that the amount of asphalt remaining attached to the surface of the corkboard as indicated at 25 42 is insufficient to properly seal the corkboard against ingress of moisture. Consequently, under such conditions, after the wall has been assembled, air and consequently water vapor will be drawn into the wall structure, resulting in the condensation of moisture therein. It is just such a condition that results in a rapid deterioration of the insulating material as set forth above.

If, on the other hand, the temperature is too low, the degree of penetration is so little as to cause improper adhesion of the asphalt to the corkboard slab, such a construction results in the separation of the asphaltic material from the insulation during use of the cabinet and consequently improper sealing of the material 14.

Such a condition is shown exaggerated in Fig. 4, wherein it will be noticed that the asphalt has not penetrated the corkboard at all and under such conditions a proper bond between the liner and the corkboard is impossible. Such a condition usually results in a shifting of the insulating material with the consequent formation of heat leaks.

As a specific example of my invention, the asphaltic compound may be a pitch-like bituminous product, or, in other words, a refined petroleum product free from filler or other material and having a softening point not less than 180° F. and not more than 200° F. I have found that with such an asphaltic compound, if the temperature of the asphalt is maintained at substantially 350° F.-365° F. during the entire act of applying the asphalt to the insulating slab, the ideal condition as indicated in Fig. 5 is obtained. That is to say, the penetration of the asphalt 40 into the insulating block 14 will be sufficient to cause a proper adhesion of the asphalt to the block and thereby obtain proper sealing thereof while at the same time it will not be great enough to substantially impair the insulating qualities of the insulating block. At the same time the asphalt will adhere to the insulating block and will produce a thick substantially smooth layer 42 of asphalt thereon having a very glossy appearance and substantially free from air spaces.

I have found that if the temperature of the asphaltic material is below approximately 350° F. when working with the specific example given above, that the degree of penetration is insuffi-

cient to cause proper adhesion of the asphaltic material to the insulating material, the result being substantially as shown in Fig. 4. On the other hand, if the temperature of the asphaltic material is allowed to rise much above 365° F., for example 375° F., then the layer of asphaltic material begins to get uneven and rough, conforming substantially to the uneven surface of the insulating block as shown in Fig. 3. At this temperature the finish is still glossy but air spaces appear therein indicating that the degree of penetration has passed the desired degree. At 400° F. and temperatures above 400° F., the finish is dull and the penetration is such as to leave substantially no layer of asphaltic material on 15 the insulating slab.

A glossy substantially smooth layer of asphaltic material free from air spaces, may be taken as an indication of proper temperature at which the asphaltic material should be applied.

There are on the market various products having substantially the properties of the asphaltic material specifically mentioned above. Some of these asphaltic materials soften at a temperature below 180° F. while others soften 25 at a temperature above 200° F. When dealing with an asphaltic material melting below 180° F., obviously the temperature at which such a material will be applied to the insulating material will be substantially lower than 350° F. Likewise, when dealing with an asphaltic material whose softening point is above 200° F., the temperature at which the asphaltic material will be applied to the insulating material will be above 365° F. With any asphaltic material, however, the temperature at which the material is applied to the insulating material should be maintained substantially at that temperature which will give a smooth glossy layer of asphalt substantially free from air spaces and properly 40 adhering to the insulating material.

While I have disclosed one specific asphaltic material and various methods by which this asphaltic material may be applied to insulating material, it should be understood that my invention relates generically to the step of controlling the temperature at which application takes place to provide a smooth glossy layer of asphaltic material on the insulating material, thereby providing proper sealing of the insulating material from the atmosphere and thereby overcoming the fault that has caused practically all refrigerator cabinet difficulties heretofore.

While the form of embodiment of the invention as herein disclosed constitutes a preferred form, it is to be understood that other forms might be adopted, all coming within the scope of the claims which follow.

What is claimed is as follows:

1. That step in the art of applying asphalt to insulating material which comprises maintaining asphalt and applying the asphalt to the insulating material at a temperature giving only sufficient penetration to cause adhesion of the asphalt to the insulating material while providing a smooth glossy layer of asphalt thereon to protect the insulation from moisture.

2. The method of coating insulating material with an asphaltic material having a softening point between 180° F. and 200° F. which comprises heating the asphaltic material to substantially 350° F.-365° F. and applying the asphalt to the insulating material while maintaining the temperature of the asphalt to be applied substantially constant at this temperature during

the entire act of applying the asphalt to the insulating material.

3. The method of coating or applying pitch-like asphaltic material to insulation which comprises heating the asphalt to a temperature above its softening point and applying the asphalt to the insulating material while maintaining the temperature of the asphalt to be applied substantially constant at the point where a substantially smooth, glossy adherent layer of asphalt is formed on the insulation.

4. The method of insulating and sealing the insulation of a refrigerator cabinet which comprises applying a coating of asphaltic material having a softening point between 180° F. and 200° F. at a temperature of between 350° F. and 365° F. to the outer surface of the inner liner; applying a slab of insulation to the outer surface of the inner liner so coated while maintaining the asphaltic material to be applied at substantially between 350° F. and 365° F.; and then applying the asphaltic material having a softening point between 180° F. and 200° F. at a temperature of substantially between 350° F. and 365° F. to the

outer surface of the slab of insulating material.

5. The method of insulating and sealing the insulation of a refrigerator cabinet which comprises applying a slab of insulating material to the outer surface of the inner liner; and applying asphaltic material to the outer surface of the insulation at a substantially constant temperature at the point where a substantially smooth, glossy adherent layer of asphalt is formed on the insulation. 5

6. The method of coating a cork insulating material with an asphaltic material having a softening point between 180° F. and 200° F. which comprises heating the asphaltic material to substantially 350° F.-365° F. and applying the asphalt to the insulating material while maintaining the temperature of the asphalt to be applied substantially constant at this temperature during the entire act of applying the asphalt to the insulating material to obtain a slight 15 but adequate penetration of the asphalt in the insulating material and a smooth glossy surface coating of the asphalt. 20

FREDERIC L. CHASE.